

Sept. 28, 1937.

C. G. MUENCH

2,094,371

FIBERBOARD

Filed Sept. 29, 1934



Witness  
Martin & Olsen:

Inventor  
Carl G. Muench  
By *Edw. Thompson*

## UNITED STATES PATENT OFFICE

2,094,371

## FIBERBOARD

Carl G. Muench, New Orleans, La.

Application September 29, 1934, Serial No. 746,112

7 Claims. (Cl. 92—39)

In the manufacture of fiber board and particularly fiber board of the type ordinarily referred to as fiber insulation board, it has been usual that such products present only a plain uniform surface which is what might be termed non-decorative. These boards are ordinarily formed as a continuous sheet, felted from a dilute suspension of fiber, on a board machine. The surface of the product thus produced is monotonously similar, a relatively uniform felted fiber appearance.

It is the object of this invention to produce a decorative felted fiber product produced as above, felted on a board machine from a dilute fiber suspension, but which will produce when properly prepared a decorative product. The product produced in accordance with the invention hereof shows on a face a self decorative effect.

Briefly, the effect referred to is achieved by first forming which might be termed fiber strings, on what are subsequently formed the fiber board so that the fiber strings are embedded and integrally incorporated in the board at a face thereof. A board thus formed is not per se a decorative product but it comprises the base product which, with another operation thereon, becomes the finished decorative product. The board with the fiber strings embedded in its face is run through a sander, or in other appropriate manner, a thin cut of fiber is removed from the face in which the fiber strings are embedded, and there then results the desired decorative material.

The inventions hereof are illustrated in the accompanying drawing wherein:

Figure 1 is a perspective view of the product hereof showing the decorative effect obtained, and

Figure 2 is a diagrammatic view of an apparatus for forming the fiber strings with subsequent formation of fiber board thereon.

In order that the invention may be readily understood, there will be first briefly described the board machine on which the product is produced in connection with which the steps of formation thereof will be described.

The board machine illustrated in Figure 2 is a type of machine now used in the manufacture of fiber insulation board. The head box 10 is supplied with a dilute suspension of fiber from supply pipe 11. The fiber stock flows from head box 10 into machine chest 12, in connection with which, baffles 13 and 14 and rotary agitator 15 serve to smooth out the flow and maintain a uniform fiber suspension.

Across the mouth of the machine chest there

are positioned mould rolls, the top roll being designated as 16 and the bottom roll as 17. It is of course understood that mould rolls 16 and 17 are covered with wire screen, not shown, and that provision is made for necessary escape of white water, or the suspension water from which the fibers have been filtered out in board formation.

In a board machine of the type above described, there must be provided seals to prevent leakage of stock between the mould rolls and the edges of the machine chest. The mold roll seals are shown at 18 and 19, and comprise strips of rubber, leather or other like flexible material. It will readily be seen that mold roll seals 18 and 19, being of flexible material, will be pressed against the surfaces of the mold rolls by the pressure of the stock in the machine chest and thus they serve to prevent leakage.

It has been found that if an auxiliary pond of fiber stock is maintained on what may be termed the wrong side of the mould roll seal, in effect a pond of stock maintained on top of the machine chest, such stock can be formed onto the top mould roll before it passes the seal. An auxiliary stock pond is illustrated at 20 adjacent to top mould roll seal 19, the auxiliary pond being fed from stock pipe 21.

As the sheet or film of fiber formed on top mould roll 16 from auxiliary stock pond 20 is, of course, quite soft since there has been no action other than gravity sheet formation, such film as it is carried down past mould roll seal 19 in the normal rotation of mould roll 16 is deformed, in fact such sheet is caused to roll up into numerous stringlike fibrous rolls as will be readily understood from a consideration of the effect of the motion of the surface of revolving mould roll 16 relative to stationary seal 19.

As the rolled up fiber strings are rolled out from under seal 19, fiber from the suspension in the machine chest immediately begins to felt out on the screen over such fiber strings. As the mould roll continues its rotation, fiber will be deposited to considerable depth over the mould roll surface, and as will be readily understood, there will emerge from between mould rolls 16 and 17 a more or less thick felted board dependent upon conditions of operation. The board produced tho will differ from ordinary board in that there will be thoroughly embedded and felted in one face thereof the fiber strings formed from auxiliary stock pond 20.

It will, of course, be understood that any desired grade or color of stock may be supplied to auxiliary stock pond 20, and that if desired, such

- pond may be subdivided across the width of the machine with different stock supplied to the different subdivisions, and that other modifications of this general nature can be made as will be understood by the skilled operator.
- 5 5 Board produced as above described, is dried in any appropriate manner and then a surface cut is taken from that surface of the board in which the fiber strings are embedded. It is, of course, understood that the surface cut may be made by 10 passing the board through a sander, a planer or the like, and that such cut shall be such that it cuts well into the section of the fiber strings. The final product produced as above described is that 15 of a fiber board with distinct markings comprising the visible sections of the fiber strings. The final product produced as above described is that of a fiber board with distinct markings comprising the visible sections of the fiber strings, which 20 according to the details of manufacture, form a contrast due to the differing arrangement of the fiber in the fiber strings, or the coloration thereof if a fiber differing from the board fiber was used 25 for the auxiliary stock.
- 25 From consideration of the above, it will readily be seen that there has been described a simple method for the manufacture of a decorative fiber board product which has a pleasing appearance, and that such product, due to the simple methods 30 employed, requires substantially no alterations of existing board machines for its production. A particularly important feature of the invention from the operating viewpoint is that to start or stop production of this decorative board, 35 it is only necessary to turn on or off the supply of auxiliary stock without other changes in operation.
- 35 The invention having been fully described above, I claim:
- 40 1. Fiber board comprising a substantially original uniformly felted main body portion, string-like fiber rolls embedded and felted into the main body portion adjacent a face thereof, the finished face thereof comprising a cut surface made up in part of longitudinal sections of such fiber rolls.
- 45 2. A fiber board having a surface made up of, in a large part, heterogeneously felted fiber, a portion of such surface comprising longitudinally sectioned sections of fiber strands felted there-

into and composed of roughly parallel longitudinally arranged fibers.

3. A fiber board the major portion of which comprises heterogeneously felted fiber, such board having included integrally therein at a 5 surface discontinuous and longitudinally sectioned groups of fibers roughly stranded with the fibers thereof lying in a generally parallel relation.

4. The method of forming a decorative fiber board wherein a portion of the fiber is caused to 10 form strandlike groups having the fibers thereof in a roughly parallel arrangement, the remainder of the fiber then felted over and including such strandlike groups, the formed board then dried and the surface incorporating the fiber strands 15 subjected to a cutting action removing the originally formed face of the board for a depth less than the depth of the strands.

5. The method of formation of a fiber sheet 20 wherein a minor fraction of fiber is felted out on a sheet forming wire and is subjected to the effect of relative motion of surfaces having the effect of rolling such felted fiber roughly into strand-like sections and subsequently the major fraction of fiber is felted out of suspension on the 25 same wire over such strand-like sections whereby such strand-like sections are integrally incorporated in a face of the formed product.

6. The method of formation of a decorative fiber sheet wherein there is formed on a felting 30 wire roughly stranded discontinuous fiber groups, in which groups the fibers are in general parallel arrangement, a pulp sheet then felted over and incorporating at a face thereof the stranded fiber groups, the complete pulp sheet then dried 35 and finally the surface in which the stranded fiber groups are incorporated removed to a depth sufficient to expose the incorporated stranded fiber groups in longitudinal cross section.

7. A fiber board comprising a felted main body 40 portion having integrally incorporated and felted therein, at a surface, elongated groups of fiber, the fibers thereof being in an approximate of parallelism, the such fiber board having had its original face, in which the string-like groups of 45 fiber are imbedded, removed to a depth to expose such elongated groups of fiber as longitudinal section thereof, and thus forming a variegated surface.

CARL G. MUENCH. 50